

G. A. HENDERSON.  
FIBROUS COMPOSITION AND PROCESS FOR MAKING THE SAME.  
APPLICATION FILED FEB. 12, 1916.

1,265,655.

Patented May 7, 1918.



# UNITED STATES PATENT OFFICE.

GEORGE A. HENDERSON, OF ST. ALBANS, WEST VIRGINIA.

## FIBROUS COMPOSITION AND PROCESS FOR MAKING THE SAME.

1,265,655.

Specification of Letters Patent.

Patented May 7, 1918.

Application filed February 12, 1916. Serial No. 77,953.

*To all whom it may concern:*

Be it known that I, GEORGE A. HENDERSON, a citizen of the United States, residing in Highland Villa, at St. Albans, in the county of Kanawha and State of West Virginia, have invented certain new and useful Improvements in Fibrous Compositions and Processes for Making the Same, of which the following is a clear, full, and exact description.

The invention relates to a new process for rendering woody particles unnatural and restoring them to their initial density and consistency in a preserved state and to the manner of their incorporation with a preservative-binder in forming building and paving structures of the class referred to in my issued United States Patent No. 1,040,321, of 1912, and my pending applications, Number 874,934, filed November 30, 1914, and Number 64,285, filed November 30, 1915. While the latter represent substantial improvement in the art, my present invention is based on my discovery that superior structures are more economically obtainable by substantial departure from the processes heretofore disclosed. Also, while in my former processes I use the waste wood from tannic acid and dye manufacturers, in whose process the wood is denatured, in the present process an incidental object is to reduce to commercial use the great quantity of hardwood heretofore discarded as waste culls of veneer plants, in which the wood is merely softened by water before shearing it into sheets of uniform thickness.

Hereinafter, in relation to this invention, by "particles" I mean woody particles of not exceeding  $\frac{1}{8}$ " in uniform thickness, shredded into various lengths and breadths graduating in irregular area aggregating  $1\frac{1}{2}$ " x  $1\frac{1}{2}$ " down to the thickness of the particles, the edges of which are beveled, ragged and torn to tatters in being shredded from the sheets of the wood sheared from the log, measured in predetermined quantities of each size in regularly descending gradations from the largest to those approximately  $\frac{1}{2}$ " x  $\frac{1}{8}$ ", forty per cent, those from  $\frac{1}{2}$ " x  $\frac{1}{8}$ " to the thickness thereof 50% to which is added 10% of particles reduced in size from the greatest thickness to those of dimensions corresponding to the thickness of the ragged edges of the particles, all impalpable dust being entirely eliminated.

By "fibers" I mean those longitudinal strands of tougher consistence than the cellular tissue by which they are surrounded in their natural state; by "pores" I mean those spaces within the wood particles walled by the fibers composing the particle, whether filled or unfilled; by "voids" I mean spaces or interstices between the separate woody particles; by "moisture" I mean a quantity of water in excess of that required to maintain the identity of the fibers as such; by "normal" I refer to the natural state or size of the particles and the natural volume of their pores before abnormal enlargement or other treatment herein referred to; as well as to the consistency and volume of the binding preservative hereinafter described, when cold, and before expanded or subjected to the treatment herein prescribed; by "bitumen" I mean a compound of pitch, natural or artificial asphalt of bituminous nature used in paving structures, and known to the trade; by "penetration" I mean the United States standard measure of consistency and density of bitumen as applied to paving structures.

In practice I have discovered that durability of such compositions is increased by the present process in which the particles are more completely, efficiently and economically denatured, pre-expanded, impregnated, contracted, bound and compressed, the graded particles more uniformly mixed and advantageously positioned in the mass, and the impregnating binder more thoroughly and uniformly disseminated throughout the mass by simultaneous accomplishment of these objects, than in the manner disclosed in the prior art, as distinguished from which the particles are, in the present process, not heated, their sap and pulp not extracted, they are not saturated with water, nor are they expanded, then dried and contracted before impregnation with their preservative-binder. On the contrary these steps are more simply and effectively taken simultaneously, that of water saturation being entirely eliminated. The destructive distillation of the cellular tissues of the particles, and the expelling of their sap and moisture content, together with maximum expansion of the pores and the consequent development of maximum absorbing efficiency of the particles, results from my employment of extreme heat, above the normal carbonizing

ing point of the bitumen, as well as that of the wood, sustained throughout such impregnation of the particles by their binder, and during partial compression of the mass, 5 as and for the purposes hereinafter described.

I have discovered that such heat, in combination with substantial vacuum created within the chamber containing it, is essential to sufficient fluidity of a quantity of bitumen in excess of that required in the completed product, which excessive quantity is temporarily needful in my process for the purposes hereinafter described, and that 10 such heat is also essential to provide the required degree of expansion of the particles, and the maximum development of their absorbing efficiency to insure perfect impregnation of the particles by their binder, as 15 well as to insure substantial reduction in the latter's quantity and consistency, in combination with simultaneous fixture of the graded particles in horizontal layers thereof, for the purpose of securing their vertical 20 positions under traffic at right angle thereto, upon which element alone the life of natural woodblock pavements is recognized to depend.

While I appreciate the fact that such heat 30 will result in volatilization of the essential oils in the bitumen, I have discovered that, as an example, the artificial asphalts adaptable to incorporation with sand and stone in paving structures, contain a prohibitive 35 quantity of such oils for use with woody particles, because of my discovery of the fact that to the extent the oily constituent is increased the bonding value of the bitumen is lessened, and that oil will not bind 40 woody particles, but on the contrary, seriously interferes even with their own mechanical clasp with each other. I have discovered that when surrounded by an excessive quantity of the bitumen, the particles, 45 when inclosed in a vacuous space, will, even in the presence of such oxygen as is expelled from the decomposing cellular tissue of particles, (which oxygen is, as quickly as formed, expelled from the chamber) not 50 ignite or carbonize when exposed to as high as 500 degrees Fahr., and that while, if this heat is sustained a sufficient length of time, the preserving and binding value of the bitumen will be thereby destroyed, yet 55 in my process such heat is applied in predetermined degree with especial regard to that required to reduce the oily constituent of the bitumen, and its normal fluidity from an excess thereof to the exact consistency 60 for practical use with woody particles in the completed product.

In my search for means of retaining essential ductility of bituminous compounds in which the oily constituent is reduced to 65 the minimum, I have discovered that the

presence of the excessive quantity thereof, when first mixed with the particles, may, in addition to providing the employed means for avoiding carbonization of the wood and bitumen by the severe heat, be advantageously utilized, in combination with such heat, and with the steam in evolution, when super-heated, as a means for absorbing pure sulfur, added in practical quantity to the other ingredients of my composition while 70 mixing them; and I have further discovered that while in the use of natural sulfur-bearing asphalts, but a comparatively small quantity of pure sulfur should be added to the mixture, yet in the use of artificial 75 asphalts the addition of this ingredient results in increased ductility of bitumen thereby made more cementitious in its relation to woody particles, and less affectable by the heat of summer or the cold of winter 80 than any bituminous compound used for paving of which I have knowledge: provided, however, the excessive quantity of oily constituent is first present to act, under the influence of severe heat, as the absorbing 85 medium of the sulfur, to be then partially eliminated by volatilization thereof.

In a further modification of my process, and as distinguished from its use in forming paving structures, I have also discovered 90 that in my manufacture of water-proofed building blocks, columns and other substitutes for timbers, in which no bitumen is used, the natural particles contain much, in addition to their fibers, that is practically 95 usable in forming such compositions,—viz., most of the hard-woods, such as beech, maple, oak and the like, contain a large percentage of pyroligneous acids, which in practice I have separated from the wood 100 by destructive distillation of its cellular tissue, in the manner heretofore described. when combined, as they do, with sulfur, in the presence of the steam expelled from the wood, hydrated sulfuric acid is formed, 105 which, in contact with casein in solution, produces a gummy mass of cementitious value. Because of the simultaneous enlargement of, and the incidental creation of vacua 110 within the pores of the particles, this substance is absorbed at once by the pores. If then this is done in the presence of approximately 500 degrees Fahr., I have discovered 115 that the particles are thoroughly water-proofed, and are ready to be compressed 120 into shape in the manner hereinafter described. In fact I have in practice impregnated the pores of hardwood with a solution of sulfur and crude pyroligneous acid, and found that the heating thereof, *in vacuo*, 125 to a temperature of approximately 500 degrees Fahr., resulted in perfect and permanent waterproofing of the wood.

In a further modification of my invention fireproofing solutions of any known con- 130

sistence may be added before or after the mass is so impregnated.

In a further modification of my invention, the building or paving structures may be reinforced by wire mesh, twisted steel rods, or other reinforcing matter placed within the structure before compression thereof.

It has been heretofore proposed to cause particles in paving aggregates bound with bituminous or other compounds to lie flat on horizontal relation to each other and to the earth, and it has been recognized that if such woody particles could be bound in a preserved state in such manner that only the ends of the fibers could be presented to the action of traffic, a much more durable product would result from the tendency of the particles to mat under the influence of such wear with less likelihood of disturbing the bond between the particles touched by traffic than if the fibers were present in the mass in variously inclined positions.

The horizontal fixture of my particles in paving structures is insured by (a) the irregular length and breadth exceeding their uniform thickness, (b) their beveled, tattered edges, (c) consequently their natural inclination to lie flat in a quantity of fluid of the consistency of water sufficient to float them until such flat, horizontal positions are assumed, (d) vibratory motion of their container during setting of the particles; (e) together with the action of the severe vacuum within which they are so positioned, and (f) the entire absence of pressure, atmospherically or otherwise, until the mass is mechanically compressed without disturbing the relative location of the particles.

A composition of such particles mixed with bitumen is more practically, than otherwise, compressed to a thickness of only two inches. If greater depth of the product is desired, such increased depth should be formed by layers of the completed product cemented together. When the pavement structure is of the form of ordinary sheet asphalt, I prefer, for the sake of horizontal or vertical presentation of all the particles to the action of traffic, as the case may be, to cut the material into blocks or slabs 36" x 36", set dodge-fashion, in the one case, and to cut the material into blocks 2" x 2" x 9" in the other case, and I have discovered that when, before placing, the blocks are painted at their edges with a sufficient quantity of the same cementing agency as that with which the particles are bound together, the blocks will adhere to each other so intimately, within a short time after being subjected to traffic, as to form substantially a monolithic pavement, the joints in which are not discernible to the naked eye.

In a modified procedure I mix predetermined percentages of bitumen and normal woody particles of various sizes, such as

described in my co-pending application Serial No. 874934, under sustained heat sufficient to destroy the cellular tissue, sap and discharge the distillates thereof and moisture from the mixer during development of the absorbing capacity and impregnation of the particles' pores by the bitumen and I lay the material on the previously prepared road base hot, gradually cool and contract it, and then compress the same, during contraction, into a sheet pavement in the manner in which sheet asphalt is laid.

I have discovered that the popular impression that the hotter, and consequently, the softer the mass is, the denser it can be compressed, when hot, is entirely erroneous as related to fibrous compositions. Even in mineral compositions mixed with hot bitumen the elements of expansion and contraction of the bitumen itself are not sufficiently guarded against in this regard, whereas with wood fiber, I have discovered that the particles do not reach the limit of their contraction until cold, and while heat is essential to render the mass sufficiently plastic to rake, spread, or otherwise handle in forming a paving structure, it may be, after being so formed, compressed preferably when thoroughly cooled to atmospheric temperature, than compressed when hot. I have also discovered that lack of regard for, and insufficient means to avoid the entrapping of air and gas bubbles within the mass during compression has been responsible for the presence of a prohibitive volume of voids in the completed product. I have discovered that plunger compression of such material in any other than an open mold is wholly impracticable, while plunger compression of such material in any mold is inefficient, in that in every case it seals the top and bottom of the mass before releasing the gas and air in its center, or giving a full opportunity to the ingredients to contract from abnormal expansion caused by their heat. I have found that even the top and bottom roller compression, adopted by me as the most practicable, in an open mold, is accompanied by unfavorable elements which are necessarily guarded against in the formation of a perfect product: viz., the tendency of such compression of the warm, plastic mass, to increase its sheet area at the sacrifice of vertical density, as well as the slight inclination of all particles toward one direction. In my process the mass in the first instance is conveyed, independent of the forwarding influence of the rollers, between them, by a foraminated belt inclosed at its surface with an end and sides completing the container for the material; after being sufficiently compressed and cooled the material passes onto a shelf inclosed at its sides, reliance for forward motion of the sheet being then had on the forwarding influence

of inversely operated reciprocating rollers through which the material then passes and is further compressed, as hereinafter described, in which operations the material is cut into slabs, and then given a back and forth serial pressure at its bottom as well as top, then crosswise, and then the reverse, during cooling, and when cold, finally compressed in a hydraulic press, simultaneously cutting the cold blocks into the desired size. I have discovered that the foramination of the plunger and plate in such molds have heretofore interfered with removal of the blocks therefrom, though aiding in the elimination of otherwise entrapped gas and air bubbles in the mass; while in the case of such small sheets of particles, stationed horizontally to such foraminations, as in my process described, this condition is avoided by the fact that the individual holes in the plunger and plate are less in area than that of the average particle forced against them.

In removing the mass from the superheated chamber as above described it would immediately ignite were it not for my provision for its cooling, in an adjoining chamber, *in vacuo*, and its emission to the atmosphere at not exceeding 200 degrees Fahr.

I have discovered that an excess of bitumen of the consistency essential for such compositions, cannot be expressed from the particles unless they are so abnormally expanded, and such expressing accomplished by severe compression when the bitumen is, by severe heat, maintained at a degree of fluidity equivalent to that of water.

In my process the relative proportions of impregnating-binder and particles are predetermined by a test of the ingredients to be used, in which the relative weights and volumes thereof in the completed product are compared with the normal particles and impregnating-binder before treatment, taking into account the reduction in weight of the particles during treatment, the reduction in the oily constituent of the bitumen in treatment, the mixing of an excess of normal bitumen to the extent of 50% of the volume required in the completed product, and regulating the pressure applied in expressing from the mass a quantity of the bitumen in exact accord with the quantity required to completely fill the contracted pores of the particles, to coat them, to fill the compressed voids between the particles, and to bind them to each other in the completed product.

Contrary to the popular means of increasing the quantity of oily constituent of the bitumen to insure sufficient resiliency in paving structures, as for example set forth in the Warren Patent No. 727,505 of 1903, I have discovered that because of the natural flexibility of my particles as compared with the inherent rigidity of sand and stone in paving structures, I may, and I prefer, in

practice, to, reduce the normal penetration of artificial asphalts used in such structures from approximately 65-70 penetration to 38-43 penetration, by the means embodying the accompanying advantages herein disclosed.

I have discovered that no bituminous compound containing water is practical for use with woody fibers, and, also, that to the extent any moisture is present at the juncture of the wood and bitumen will adhesion be seriously interfered with. I have also discovered that my particles, when all moisture is removed from their pores, will atmospherically absorb from 10 to 20 per cent. thereof, depending on the atmosphere; hence the advantage of completely drying the pores and surfaces of the particles, simultaneously with their impregnation with moisture resisting solutions.

I have also discovered that any impalpable powder, such as wood dust, or even Portland cement, seriously interferes with the adhesive efficiency of the bitumen to the surface of, and the walls of the pores within, the particles; and in practice I prefer to eliminate it entirely.

In recognition of the explosive element of a mixture of 1% oxygen with 2% hydrogen, when ignited by a spark, in combination with simultaneous creation of both by the destructive distillation of the cellular tissues of particles, due regard shall be given in carrying out my process to create the maximum exhausting efficiency of the fans used for creating the vacuum referred to, in combination with such aid thereto, and the accompanying safe-guard, due to the reduction in volume of the steam in evolution by exhausting it from the particles and chamber containing it in a dry and superheated condition.

My invention can be readily understood by reference to the accompanying drawings, which will now be described, it being premised, however that various changes may be made in the apparatus here illustrated as one means for carrying out the steps of my process, without departing from the spirit and scope of the invention as defined in the accompanying claims.

Figure 1 is a view partially in section of apparatus for shearing, shredding, grading, measuring and mixing the particles in combination with apparatus in horizontal section for mixing the ingredients and impregnating mechanism, portions being broken away for the purpose of better illustration; Fig. 2 is a vertical cross section of mixing apparatus shown in Fig. 1; Fig. 3 is an end view of impregnating apparatus in vertical section; Fig. 4 is a side elevation of cooling apparatus, with vacuum attachment, Fig. 5 a cross-sectional end view of compression apparatus, Fig. 6 a side view, in section,

thereof, and Fig. 7 is a side elevation in section of a hydraulic press.

Referring to the drawings by numerals, in carrying out my invention, the wood is sheared into sheets from the log 1 anchored by clamp 1<sup>a</sup>, revolved by pulley 1<sup>b</sup> driven by belt 1<sup>c</sup>, the log being in engagement with fixed knife 2. The sheets 3, of the desired thickness, are deposited into hopper 4<sup>a</sup> of shredding machine 4, in which the sheets are reduced to particles by shredding mechanism operated by pulley 4<sup>b</sup> driven by belt 4<sup>c</sup>. The particles are conducted from the shredding machine through chute 4<sup>a</sup> and deposited onto screen 5, within which is spread mesh which will permit the passage of particles of the size 1" x  $\frac{1}{4}$ " graduating down to those of an average size corresponding with the thickness of the ragged edges of the particles. Screen 5 is slightly inclined from horizontal and is designed to be given a vibratory motion, which will cause the particles which will not pass its mesh to be worked to the top of the screen and deposited into re-shredding machine 6, operated by pulley 6<sup>a</sup>, driven by belt 6<sup>c</sup>, in which these larger particles are cut into smaller sizes and returned to screen 5 by belt conveyer 7<sup>a</sup> after being deposited through chute 6<sup>a</sup> into container 7. Screens 5<sup>a</sup> and 5<sup>b</sup> preferably contain mesh which will permit of the passage, first, of particles in size  $\frac{3}{4}$ " x  $\frac{3}{16}$ " graduating downwardly, and secondly, of particles in size  $\frac{1}{2}$ " x  $\frac{1}{8}$ ", graduating downwardly, those failing to pass screens 5<sup>a</sup> and 5<sup>b</sup> being conducted by their inclination from horizontal into measuring boxes 8<sup>a</sup>, and being in the minority of the mass; those passing screen 5<sup>b</sup> shall pass screen 5<sup>c</sup> in major proportion of the mass, and are likewise conducted to measuring box 8<sup>a</sup> as shown. The particles are then measured in predetermined quantities of each of the several grades from the largest, viz.,  $\frac{3}{4}$ " x  $\frac{1}{4}$ " by the thickness of the sheets, in regular descending gradations down to the size  $\frac{1}{2}$ " x  $\frac{1}{8}$ " 40% thereof; those from  $\frac{1}{2}$ " x  $\frac{1}{8}$ ", to the thickness thereof 50%, while approximately 10% of smaller particles in the mass is secured as a result of adjusting the shredding machine to produce practically this quantity in the shredding of the sheets into particles. The particles are then mixed in the common chute 8, by which they are conducted to a measuring container 11, through which in proportions in relation to that of the impregnating-binder yet to be referred to, the particles are discharged into mixing apparatus 12, through gate 12<sup>a</sup>. The impregnating-binder hereinabove described, is preferably heated to sufficient fluidity in kettle 9, measured in predetermined proportion in relation to the proportion of particles, as described, in measuring kettle 10, and dis-

charged through cock 10<sup>a</sup>, simultaneously with the particles, into the mixer 12, through pipe 10<sup>b</sup>, or otherwise. Chamber 12 is nested within oven 13, surrounding substantially three-fourths of the mixing 70 chamber 12, in which oven heat is supplied by a furnace, the heat from which preferably generated by burning gas, or oil, is conducted by exhaust fan 13<sup>a</sup> in stack 13<sup>b</sup>, so as to partially surround the inclosed section of the mixer 12, and at the point 13<sup>c</sup> be sucked into and through the inner chamber of mixer 12, in direct contact with the composition therein being agitated and mixed by the operation of agitating blades 12<sup>a</sup> 80 anchored to central shaft 12<sup>b</sup> revolved by pulley 12<sup>c</sup> driven by belt 12<sup>d</sup>. The mouth of mixer 12 extends from a point in the shell of said mixer extending externally of the oven 13, which mouth 12<sup>e</sup> is equipped 85 with air-tight gate 14<sup>b</sup>, in housing 14<sup>a</sup>, toward which the material in the mixer 12 is conducted by the peculiar shape of the agitating blades 12<sup>a</sup>. Gate 14<sup>b</sup> may be operated by hand, care being taken that at least 90 one-fourth of the space within the housing 14<sup>a</sup> is filled with the material when the gate is turned to admit the material within impregnating chamber 14. If, in accord with the modification of the invention hereinabove described the composition is to be laid in monolithic sheet form and not manufactured into blocks, the material is, at this point deposited through gate 14<sup>b</sup> onto the previously prepared base of the roadway, 95 but in this event, the material is permitted to remain in drum mixer 12 until the particles have exhausted their absorbing capacity and become impregnated with the bitumen in the manner described. Upon 100 reaching this chamber the mass is dropped onto baffle plate 14<sup>c</sup>, the first of a series thereof, anchored in an inclined position within chamber 14, to which plates may be attached off-sets which act to turn the mass, 105 and to expose the particles thereof to the heat and vacuum influences within chamber 14 hereinafter described, in the fall of the material from the top of the chamber 14 to its bottom. Between the baffle-plates, 110 as shown, endless conveyers 14<sup>d</sup>, operated by cog or sprocket connection with common shaft 14<sup>e</sup> are revolved on rollers 14<sup>m</sup>, 14<sup>m</sup>, to which conveyers are attached buckets 14<sup>a</sup>, 14<sup>d</sup> designed to pick up the 115 material at the bottom of the chamber 14, lift it to its top and drop it through the heated vacuum of the chamber, over the baffles 14<sup>c</sup> to the bottom of the chamber in a sufficient number of such operations to 120 expose each of the particles to the influence of the heat and vacuum within the chamber 14, hereinafter described, for the purposes hereinabove set forth.

Chamber 14 is preferably constructed of 130

heavy steel, and its lower curvature incased within firebrick 15<sup>c</sup>. It is preferably heated by two furnaces the heat from which converge at its longitudinal center and is exhausted through stack 15<sup>d</sup>. Chamber 14 is partially nested within the furnaces 15<sup>a</sup> 15<sup>a</sup> and shell 15, 15, within which furnaces 15<sup>a</sup> any suitable fuel may be deposited through doors 15<sup>b</sup> 15<sup>b</sup> and burned to heat the contents of chamber 14 to approximately 500 degrees Fahr. Exhaust stack 14<sup>e</sup> leading from chamber 14 to condenser 14<sup>k</sup> is equipped with a powerful exhaust fan 14<sup>h</sup> in housing 14<sup>i</sup>, designed to create substantial vacuum within chamber 14. The operation of the above mechanism, and the subjection of the ingredients to the influences mentioned, therein, results in the maximum enlargement of the particles, and expansion of their pores, the complete change in character of the matter theretofore forming its sap, cellular tissue and moisture, and in its extraction and removal from the particles, the development of maximum absorbing efficiency of the pores, and their complete impregnation with bitumen present and surrounding them in excessive quantity, and also results in the reduction of the oily constituent of the bitumen, to render the bitumen of practical plasticity and binding value in the completed product, as well as the reduction of the plastic bitumen to a state of extreme fluidity, in which condition it, together with the particles which it surrounds, is deposited within chamber 14 onto endless conveyer 16<sup>b</sup>, which conveyer is foraminated and is revolved by cog or sprocket wheel 16<sup>f</sup> (shown in Fig. 8) around drums 16<sup>e</sup>—16<sup>e</sup>. Compressor rollers 16<sup>a</sup> are revolved by the action of their axles extending through the walls of chamber 14 and oven 15, in air tight bearings, and are anchored in retaining bearings, within which they revolve, riveted to the inside walls of chamber 14,—while compressor-rollers 16<sup>s</sup> are adjustable by hand manipulation in such manner as to regulate the last pressure given to the mass before emission from chamber 14, the series of compressions given by all of these rollers, revolving inversely as to conveyer 16<sup>b</sup>, of reciprocating size, speed and direction, being designed to express from the abnormally enlarged pores of the heated particles, the excess quantity of bitumen hereinabove referred to, leaving within the pores of the particles as they emerge from chamber 14 an insufficient quantity of such bitumen to fill them, but sufficient, in their subsequently contracted state, to completely fill them, to coat them, to fill the compressed voids between the particles and to bind them to each other. The bitumen expressed in the compression just referred to is precipitated into the bottom of chamber 14, inclined downwardly at this point, toward, and is emitted

through, outlet pipe 16<sup>c</sup> for use as a by-product. 16<sup>d</sup> is a man-hole for use in repairing the mechanism within chamber 14. The space between rollers 16<sup>s</sup> while normally opened, is completely closed and air-tight by reason of the severe compression of the mass between the rollers at this point. The products of distillation, as well as the fumes from the heating bitumen are conducted through exhaust pipe 14<sup>g</sup> to condenser 14<sup>k</sup> where they are entrapped and reclaimed to be subsequently used as by-products.

For a distance of approximately six feet from the innermost end of conveyer 16<sup>b</sup> the foraminated belt thereof is by proper mechanism, given a sidewise vibratory motion, the material falling thereupon at this point being inclosed by an end piece and two sides of steel construction, whereupon by such vibration and shaking of the conveyer, before the material thereon reaches the first of the series of compressor rollers 16<sup>a</sup> the particles by reason of being shredded and cut in the shape hereinbefore specified, as well as because of their feather edges, will be found to assume flat horizontal positions in relation to the belt which action is aided in the tendency of the fluid bitumen to sink through the mass on the conveyer by reason of its extreme fluidity and excessive quantity.

Endless belt 16<sup>b</sup> extends through the walls of chamber 14 and oven 15 and beyond and within cooling chamber 17 immediately adjoining, in which no heat is present other than that arising from the hot mass conveyed thereinto by conveyer 16<sup>b</sup>. Cooling chamber 17 is also equipped with a powerful exhaust fan 17<sup>a</sup> operated by pulley 17<sup>b</sup> in engagement with belt 17<sup>c</sup>, for creating and maintaining within chamber 17 substantial vacuum, to prevent ignition of the hot mass before being sufficiently reduced in temperature. Within chamber 17 the mass is further compressed by rollers 17<sup>d</sup> without disturbance of the relative positions of the particles within it, and the material is designed to remain within said chamber 17, in its course through it, a sufficient length of time to reduce the temperature to approximately 200 Fahr., and the depth of the mass to approximately 4 $\frac{1}{4}$ " before emission through its mouth 17<sup>e</sup>, which is closed by the passage of material therethrough in being compressed at that point to the thickness of approximately 4".

Whereupon compression continues, at atmospheric temperature, by a continuation of endless belt 16<sup>b</sup> through two sided trough 18, and reciprocating rollers 18<sup>a</sup> 18<sup>a</sup> which serve to reduce the thickness to approximately 3 $\frac{1}{4}$ " by the time the mass is at approximately 150 degrees Fahr., when at the point 18<sup>b</sup> the foraminated conveyer belt 16<sup>b</sup> turns on drum 16<sup>e</sup> leading toward chamber

14. Referring to the enlarged detail, Fig. 8, 18 designates a stationary trough of preferably steel construction, immediately next to the inversely operating rollers 18<sup>a</sup> 18<sup>a</sup> intervening between endless conveyer 16<sup>b</sup> and trough 18. The material being conducted to the rollers 18<sup>a</sup> by the operation of endless conveyer 16<sup>b</sup>, is of sufficient solidity to bond its particles together to be pulled 10 through and between rollers 18<sup>a</sup> by their revolving action, much the same as a cloth is pulled through the space intervening between the rollers of a clothes wringer. Rollers 18<sup>a</sup> are of exactly the same circumference, 15 revolved by the mechanism more in detail shown in Fig. 7, in which 18 designates the sides to the trough, 18<sup>a</sup> the rollers referred to, 18<sup>b</sup> cog wheels which mesh with each other in reciprocating action, driven by bevel 20 cogs 18<sup>c</sup> 18<sup>c</sup> connected with suitable power. Longitudinally of the rollers 18<sup>a</sup> a knife-like blade 18<sup>c</sup> extends the length thereof, and is preferably of heavy construction, extending at right angles to the center of the 25 rollers 1 $\frac{1}{2}$ " in depth. Rollers 18<sup>a</sup> are each preferably 36" in circumference and are so revolved that the knives 18<sup>c</sup> 18<sup>c</sup> will converge as they pass each other not more than  $\frac{1}{2}$ " apart in cutting the sheet as it passes 30 through the rollers 18<sup>a</sup> which are designed to further compress the material from 3 $\frac{1}{2}$ " to 3" in depth. The material when first compressed in chamber 14 is designed to be retained by the two sides of the trough containing conveyer 16<sup>b</sup>, which two sides are 35 36" apart, so that the blocks when first cut by the knives 18<sup>c</sup> shall be of the size 36" x 36" x 3". By the pressure of material behind them the blocks are pushed forward 40 on trough 18 until they reach a conveyer passing between compression rollers revolved in a direction at right angles to rollers 18<sup>a</sup>, which conveyer is designed to move in a direction at right angles to trough 18, 45 in which latter operation the blocks are further compressed to approximately 2 $\frac{3}{4}$ " in thickness and at the same time are cut as in the former manner described to a size 18" x 36". The blocks are then conveyed to 50 an endless conveyer which moves them in the reverse direction to that in which they were conducted when first cut into blocks, and are in this operation again cut into sizes 18x9 inches and compressed to approximately 2 $\frac{1}{2}$ " in thickness. The blocks, 55 while still retained in a trough 36" wide, but therein fitted together, are rolled in a direction the reverse to that in which they were conveyed when cut the second time, and then compressed to approximately 2 $\frac{1}{4}$ ", the speed of the conveyers and the time elapsing between that at which they emerged from cooling chamber 17 until reduced to the thickness of 2 $\frac{1}{4}$ " being sufficient to cool 60 65 the mass throughout its depth to that of at-

mospheric temperature, whereupon the blocks are placed in a mold and subjected to hydraulic pressure to reduce their thickness to 2". It is obvious that the blocks when placed in this mold may be of any practical size, but in practice I prefer that five such blocks each of the size 18" x 9" x 2 $\frac{1}{4}$ " be placed adjoining each other in a mold of an exact size to contain them. In the described cutting of the sheet into blocks the 70 blades attached to the compressor rollers are at each revolution thereof damped with water and coated with Portland cement or other dust, which thereafter prevents the sticking together of the blocks during subsequent compression together, this being primarily due to the severance of the superior bond between the particles in the various blocks at the point of cutting. Likewise the surfaces of all compressor rollers 80 except those in chambers 14 and 17 are, as shown by the water and dust containers 18<sup>d</sup> in Figs. 7 and 8 so damped and dusted to avoid sticking, or "picking up" of the mass during compression and handling. Likewise the inside surfaces of the mold in the hydraulic press are so treated before the blocks are therein placed. 90

It is obvious that the blocks when reduced to the size 9" x 18" x 2" may be, while being 95 so reduced from their thickness of 2 $\frac{1}{4}$ " to 2", in the hydraulic press, or afterward, further cut, by known mechanism, under hydraulic or other pressure, into blocks of smaller size. In practice I prefer to cut 100 one block 9" x 18" x 2" into eight blocks 2" x 2" x 9", in one operation, an allowance of one inch being made for further lateral compression, and space for the knife blades intervening in this operation. 105

It is also obvious that the material thus produced may be, by interfering with the longitudinal positions of the particles, carried to a roadway and laid while still hot after passing through the cooler 17, as hereinbefore set forth; or the mass may be compressed into slabs of any size and thickness not exceeding 2" in the manner herein described, or the material may be cooled to atmospheric temperature upon being emitted 110 from cooler 17, stored and then reheated at point of construction for use in being spread and rolled on a previously prepared road base in the manner in which mixtures of asphalt and sand have been heretofore laid. 115 120

I claim:

1. The process of manufacturing a composition of matter for paving purposes consisting in shearing, then shredding wood into beveled, ragged edged particles of substantially uniform thickness of not exceeding  $\frac{1}{8}$ " and of irregular lengths and breadths graduating in descending scale of sizes from those approximately 1" x  $\frac{1}{4}$ " to  $\frac{1}{2}$ " x  $\frac{1}{8}$ ", measuring and mixing 40% thereof with 50% 125 130

of those in sizes graded from  $\frac{1}{2}'' \times \frac{1}{8}''$  to a cube whose diameter is the thickness of the particles, mixed with 10% of sizes graded from that of the largest cube to those of dimensions corresponding to the average thickness of the ragged edges of the particles; then mixing particles *in vacuo* with a preheated bitumen of approximately 70 standard penetration, in quantity approximately 50% in excess of that required in the completed product; then agitating the mixture while strongly heated a predetermined length of time to partially volatilize the oil of the bitumen to reduce such penetration to approximately 40, to abnormally enlarge the particles and to separate and expel from their expanded pores all moisture, sap, essences, cellular tissue and pulpy matter, by destructive distillation thereof, and, by the influence of the fan creating the vacuum, expelling from the chamber containing them, all such products, together with the fumes from the heated bitumen, simultaneously impregnating the expanded pores of the particles, by their absorption of the melted bitumen; then draining superheated bitumen through the particles, during vibration of their container, to settle the particles horizontally; then, when still heated to sufficient fluidity, expressing the excess bitumen from the particles, retaining in their expanded pores merely enough to completely fill them when subsequently contracted, to coat them, to fill the voids between the particles when finally compressed, and to bind them to each other; then cooling the mass and gradually compressing the same into shape, during and after contraction of the ingredients, substantially as described.

2. The process of manufacturing compositions in which graded sizes of flat particles of uniform thickness with beveled ragged edges are mixed with sulfur and then, under the influence of heat, with an excessive quantity of preheated bitumen of oily constituency; then exposing all parts of the mixture to the influence of strong heat *in vacuo* to reduce the volume of oily constituent in the bitumen, during its absorption of the sulfur, and to reduce the bitumen to a state of extreme fluidity, simultaneously enlarging, abnormally, the particles, and expelling therefrom, and from the chamber containing them, all moisture, essences and cellular tissue by destructive distillation thereof, and impregnating the expanded pores with, by their absorption of, the bitumen, then draining the excess of bitumen through the particles during vibration of their container, to set or settle the particles horizontally of the earth; then expressing a predetermined quantity of bitumen from the mass by compression thereof, then removing the mass from the influence of heat, and partially compressing the same while cooling *in vacuo*;

then exposing the mass to atmospheric temperature, and while further cooling, applying a series of reverse and transverse roller compressions at its bottom and top surfaces; then, when cold, further reducing its thickness by compression, and simultaneously cutting the same into blocks, substantially as described.

3. The method of producing a composition in which graded sizes of flat particles of wood of uniform thickness and ragged edges are mixed with bitumen and exposed to the influence of a temperature of approximately 500 degrees Fahr. *in vacuo* to abnormally enlarge the particles and to separate all moisture, sap, pyroligneous acids, and pulp from their expanded pores by destructive distillation of the products, simultaneously, by sufficient agitation, exposing the bitumen to the absorbing capacity of the expanded woody particles during evolution of dry, superheated steam from the mass; removing, through the agency creating the vacuum, the unabsorbed fumes and steam arising therefrom; then cooling the mass *in vacuo* and during and after contraction of the particles, compressing the same into shape, substantially as described.

4. A method of producing a composition of graded woody particles mixed in a chamber with bitumen while strongly heated, sufficient in degree to abnormally expand the particles of wood and to separate all moisture, essences, pyroligneous, and other acids and pulp therefrom; agitating the mass in the chamber to expose the bitumen to the absorbing capacity of the woody particles; impregnating the expanded pores of the particles by their absorption of the preservative-binder so formed, removing from the chamber containing it all unabsorbed steam and fumes arising from the material; then exposing the mass to atmospheric temperature, and then compressing the same into shape during and after contraction of the particles, substantially as described.

5. The method of producing a paving structure of monolithic character in which graded sizes of flat woody particles of uniform thickness, but with ragged edges are mixed, under the influence of heat with a pre-determined quantity of preheated bitumen, and then subjected to sufficient heat to abnormally enlarge the pores of the particles and to expel therefrom all moisture, essences and cellular tissue by destructive distillation thereof, the particles being simultaneously impregnated by their absorption of the molten bitumen; then partially compressing the mass when spread upon a previously prepared road base, during the cooling and contracting of the ingredients, to substantially fifty per cent. of the thickness of the uncontracted, uncompressed mass when first so spread, the final compression

of the sheet being had by transverse action of the rollers thereon after the mass is thoroughly cooled, substantially as described.

6. A fibrous composition consisting of 5 woody particles of uniform thickness and irregular lengths and breadths, impregnated and bound by bitumen in planes substantially parallel to each other.

7. A fibrous composition consisting in 10 graded sizes of woody particles of uniform thickness and irregular lengths and breadths, with beveled and ragged edges, from which particles have been removed sap, cellular tissue and moisture, impregnated with bitumen, and compressed into 15 shape, substantially as described.

8. A fibrous composition consisting of 20 woody particles with beveled and ragged edges, of uniform thickness, shredded into various lengths and breadths graduating in 25 irregular area varying from  $1'' \times \frac{1}{4}''$  down to dimensions corresponding with the thickness of the particles, mixed in predetermined quantities in regularly descending 30 gradations from the largest to those approximately  $\frac{1}{2}'' \times \frac{1}{8}''$  forty per cent.; those from  $\frac{1}{2}'' \times \frac{1}{8}''$  to dimensions corresponding with the thickness thereof, 50%; those of 35 particles in size graduating from all of the greatest thickness to those of dimensions corresponding to the thickness of the ragged edges of the particles, 10%, from which particles have been removed sap, cellular tissue and moisture, impregnated with a cementitious wood preservative and compressed into shape substantially as described.

9. A fibrous composition consisting in 40 graded woody particles of uniform thickness and irregular lengths and breadths with beveled and ragged edges, from which particles have been removed sap, cellular tissue and moisture, coated and impregnated with

a wood preservative of cementitious nature and compressed into shape.

10. A paving block of fibrous composition 45 consisting in graded woody particles of uniform thickness and irregular lengths and breadths, with beveled and ragged edges, from which particles have been removed sap, cellular tissue and moisture, impregnated with bitumen in planes substantially parallel to each other, and cut so that its breadth is that of the thickness of the compressed sheet of which it formed 50 a part.

11. The method of producing a monolithic paving structure, consisting in chipping wood into particles of various shapes and graded sizes; then coating the particles in a drum with preheated bitumen, through 60 which bitumen under sustained heat and during agitation of the mass, the cellular tissue, sap and moisture in the particles are destructively distilled and then expelled from the drum, simultaneously exhausting 65 the absorbing capacity of the particles with the heated bitumen; then depositing the mass onto a previously prepared road base and compressing the same into shape.

12. A monolithic pavement structure 70 consisting in graded woody particles of uniform thickness, and irregular lengths and breadths, from which have been removed sap, cellular tissue and moisture, impregnated and coated with a cementitious preservative and compressed into shape.

In testimony whereof I have affixed my signature in the presence of two witnesses, the twenty-second day of January, 1916.

GEORGE A. HENDERSON.

Witnesses:

L. J. WHITE,  
C. W. ZERKLE.

Copies of this patent may be obtained for five cents each, by addressing the "Commissioner of Patents, Washington, D. C."